

## UNITED STATES PATENT OFFICE

2,084,154

## PROCESS OF MAKING COPPER POWDER

Raymond P. Lutz, Oak Park, Ill., assignor to  
 Western Electric Company, Incorporated, New  
 York, N. Y., a corporation of New York

No Drawing. Application January 7, 1936, Serial  
 No. 57,967

12 Claims. (Cl. 75—117)

This invention relates to a process of making copper powder.

On account of the high ductility of copper, it is extremely difficult to pulverize copper by grinding. It appears that in grinding copper by processes which in less ductile metals would result in a reduction of the particle size, the ductility of the copper causes particles thereof to elongate, flatten, or distort, so that it has been almost impractical to obtain a fine or impalpable copper powder by grinding.

An object of the present invention is to provide an effective and efficient process of making copper powder.

In accordance with one embodiment of the invention the copper powder containing sludge from a copper wire drawing machine is treated with a non-corrosive solvent to liberate the copper particles after which the particles are separated from the solution preferably by means of a centrifugal filter.

In the drawing of a copper wire it is customary to use a wire drawing compound comprising fat and soap dispersed in water to lubricate the dies and capstan of the machine. During the drawing operation fine particles of copper are abraded from the wire and these particles together with some of the spent drawing compound settle to the bottom of the machine and form a sludge. Heretofore this sludge was either discarded or subjected to a burning and melting treatment from which the copper was recovered in the form of cast bars.

The recovery of the copper in powder form from the sludge presents numerous difficulties. Some solvents for the sludge attack the copper and corrode it while others form slimes which prevent satisfactory separation of the copper powder.

A satisfactory solvent must have a slight affinity for water since the sludge contains a small amount of water. It must also be a solvent for fats and copper soaps which are present in the sludge. The copper soaps unless dissolved form a slime from which it is impractical to separate the copper powder. The solvents which possess the necessary properties for this process are chlorinated hydrocarbons such as ethylene dichloride or trichlorethylene, ethers such as di-chlorethyl ether, or ketones such as diethyl ketone or methyl propyl ketone. If the solvent is filtered off the copper powder in such a manner as to leave the powder moist as for instance in a filter press it must be dried in a heated non-oxidizing atmosphere as an inert gas, a

vacuum or in a heated reducing atmosphere such as a hydrogen atmosphere at a temperature of approximately 500° F. to obtain a non-oxidized copper powder. To avoid the use of such an atmosphere, it is preferable to use a centrifugal filter by means of which the solvent may be removed and the copper powder dried without material oxidation.

In practising the invention a quantity of the sludge from a wire drawing machine is mixed with a quantity of the solvent and the mixture is thoroughly agitated. While continuing the agitation the mixture is supplied through a suitable conduit to a centrifugal separator which retains the copper powder and expels the solvent. When a suitable amount of copper dust has accumulated in the centrifuge the supply of the mixture is interrupted and a small amount of clean solvent is introduced into the centrifuge to wash the copper powder of any remaining impurities. The powder is then dried in the centrifuge. In this manner the copper powder is dried by centrifugal force without any appreciable aeration of the powder which would rapidly oxidize the fine powder.

It will be understood that the nature and embodiments of the invention herein described are merely illustrative and that many changes and modifications may be made therein without departing from the spirit and scope of the invention.

What is claimed is:

1. A method of producing copper powder which comprises drawing a copper wire with a fat and soap drawing compound whereby a copper containing sludge is formed, treating the sludge with a non-corrosive solvent which will not form a slime, and filtering the copper powder from the solution.

2. A method of producing copper powder which comprises drawing a copper wire with a lubricating drawing compound whereby a copper containing sludge is formed, treating the sludge with a non-corrosive solvent which will not form a slime, and filtering the copper powder from the solution.

3. A method of producing copper powder which comprises drawing a copper wire with a lubricating drawing compound whereby a copper containing sludge is formed, treating the sludge with a chlorinated hydrocarbon to dissolve the drawing compound and copper soaps, and separating the copper powder from the solution.

4. A method of producing copper powder which comprises treating the sludge from a copper wire

15

20

25

30

35

40

45

50

55

drawing machine or the like with a chlorinated hydrocarbon to dissolve the soluble constituents, and filtering the copper powder from the solution.

5. A method of producing copper powder which comprises treating the sludge from a copper wire drawing machine or the like with a solvent for the soluble constituents, and separating the copper powder by filtering the solution.

10. A method of producing copper powder which comprises treating the sludge from a copper wire drawing machine with a solvent for the fluid constituents and copper soaps, and separating the copper powder from the solution by a centrifugal filter.

15. 7. A method of producing copper powder which comprises treating the sludge from a copper wire drawing machine with a solvent for the fluid constituents and copper soaps, and separating and drying the copper powder by a centrifugal

20 filter.

8. A method of producing copper powder which comprises mixing the sludge from a copper wire drawing machine with a solvent for the fluid constituents and copper soaps, supplying the 25 mixture to a centrifugal filter, interrupting the supply of the mixture and supplying clean solvent to the copper powder, and drying the copper powder by centrifugal force.

9. A method of producing copper powder which comprises treating a sludge containing copper powder, water, fat and copper soaps with chlorinated ethylene to dissolve the soluble constituents and filtering the copper powder from the 5 solution.

10. A method of producing copper powder, which comprises treating a sludge containing copper powder, fat and copper soaps with a solvent selected from the group of a chlorinated hydrocarbon, a chlorinated ether, or a ketone to dissolve the soluble constituents and filtering the copper powder from the solution.

11. A method of producing copper powder, which comprises treating a sludge containing 15 copper powder, water, fat, and copper soaps with a chlorinated ether to dissolve the soluble constituents and filtering the copper powder from the solution.

12. A method of producing copper powder, 20 which comprises treating a sludge containing copper powder, water, fat and copper soaps with a ketone to dissolve the soluble constituents and filtering the copper powder from the solution.

25

RAYMOND P. LUTZ.